

Nov. 8, 1949

P. H. CARNELL

2,487,306

TREATMENT OF LUBRICATING OILS

Filed May 24, 1946



## UNITED STATES PATENT OFFICE

2,487,306

## TREATMENT OF LUBRICATING OILS

Paul H. Carnell, Bartlesville, Okla., assignor to  
Phillips Petroleum Company, a corporation of  
Delaware

Application May 24, 1946, Serial No. 671,990

12 Claims. (Cl. 196—39)

1

This invention relates to the treatment of lubricating oils to improve their properties. In one of its aspects it relates to the treatment of natural and/or synthetic polymerized olefin-type lubricating oils to effect an improvement in their properties. In another aspect it relates to the treatment of such oils to increase their viscosity or viscosity index or stability, or a plurality of said properties.

The prior art on the refining of lubricating oils with anhydrous liquid hydrofluoric acid shows (Frey U. S. Patent 2,378,762) that paraffinic, mixed-base or asphalt-base lubricating oil stock is improved by contacting such stock, dissolved in a low-boiling paraffin, with anhydrous liquid hydrofluoric acid and an alkylating agent or agents, such as olefins, cracked gasoline, alkyl halides, especially the nonprimary alkyl halides, alcohols, especially the non-primary alcohols, and unsaturated cyclics to form compounds of increased hydrogen-to-carbon ratio.

The principal object of the present invention is to provide a novel and an improved method of improving lubricating oils. Another object is to provide a method of improving natural lubricating oils. Another object is to provide a method of improving mixed-base lubricating oils. Another object is to provide a method of improving synthetic lubricating oils produced by polymerizing olefins. Another object is to provide a method of increasing the viscosity index of lubricating oils. Another object is to provide a method of increasing the viscosity of lubricating oils. Another object is to provide a method of increasing the stability of lubricating oils. Another object is to increase the viscosity, viscosity index and stability of mixed-base lubricating oils. Another object is to improve the properties of lubricating oils, particularly the mixed-base lubricating oils, with a minimum of loss of oil in the form of acid-soluble material. Another object is to provide a process of the foregoing type which is simple and economical to carry out. Another object is to provide a process of the foregoing type which involves low consumption of chemicals and a maximum recovery of lubricating oil. Numerous other objects will more fully hereinafter appear.

2

The accompanying drawing portrays diagrammatically one arrangement of equipment which may be used for carrying out the present invention.

5 Broadly speaking, my invention is a process of improving lubricating oil which comprises contacting the lubricating oil with substantially anhydrous liquid hydrofluoric acid and with a naphthene at elevated temperature and pressure for 10 a period of time sufficient to produce a substantial improvement in the properties of said lubricating oil, and recovering the treated lubricating oil from the resulting reaction mixture.

15 While any naphthene may be employed, I almost invariably use those naphthenes which are saturated cyclic hydrocarbons containing at least one saturated 5- or 6-carbon atom-membered ring. While the polycyclic naphthenes may be used, I prefer the monocyclic naphthenes which 20 are derivatives of cyclopentane and cyclohexane. Examples of monocyclic naphthenes which may be satisfactorily employed are cyclopentane, methylcyclopentane, cyclohexane and methylcyclohexane.

25 An example of a bicyclic naphthene is decalin (decahydronaphthalene) which embodies two fused or condensed cyclohexane rings. Other examples of bicyclic naphthenes are dicyclopentyl and dicyclohexyl. While polycyclic naphthenes having more than two saturated rings 30 may be employed, monocyclics are more frequently used in commercial practice.

The exact nature of the chemical changes that occur in the treatment of the present invention 35 is not known at the present time, but it is believed that alkylation is the principal reaction.

The lubricating oil treated in accordance with the present invention may be any hydrocarbon lubricating oil. Generally, it will be a natural lubricating oil, that is a lubricating oil derived from naturally occurring crude oils in known manner. The lubricating oil may be either a paraffin-base oil, a mixed-base oil or an asphalt-base oil. Generally speaking, I prefer to treat mixed-base oils in accordance with my invention since mixed-base lubricating oils may be deficient in certain respects as compared with paraffin-

base oils, although mixed-base oils possess certain advantages not possessed by paraffin-base oils. While my invention is generally applied to natural lubricating oil, it may also be applied to synthetic hydrocarbon lubricating oil especially the synthetic oil produced by polymerizing low-boiling aliphatic olefins.

The oil treated in accordance with the present invention displays improved properties over the original untreated oil. One property that is improved is the viscosity index. Oil treated in accordance with the present invention has a substantially higher viscosity index than the original oil. The absolute viscosity of the oil may be increased by the treatment of the present invention, may be substantially unaffected, or may be slightly lowered. In general, the stability of the oil is increased by treatment in accordance with my invention. The pour point may be increased slightly or may be the same as that of the untreated oil. Generally speaking, the gravity of the oil product of my invention is slightly above that of the initial oil. The color may be somewhat darkened by the treatment, but it is preferred that the treatment be so conducted that this darkening is not appreciable.

From this disclosure those skilled in the art will be able to conduct the treatment of the present invention in such manner as to secure the desired improvement in the properties of the oil. Reference is made particularly to the examples given below wherein different conditions of treatment and different naphthenes were employed with varying results.

The elevated temperature at which the treatment of this invention is carried out may vary within quite wide limits. Generally speaking, it will fall within the range of from 40 to 300° C. More commonly, it will be within the range of from 100 to 200° C. A temperature of from 140 to 170° C. is preferred and is used in the examples.

The pressure likewise may vary widely, but should be sufficient to hold the hydrofluoric acid and the hydrocarbons in the liquid phase throughout the reaction. Generally speaking, the pressure may range from 600 to 2000 pounds per square inch.

The contact time, i. e., the time of residence of the reaction mixture in the reaction zone under the conditions of temperature and pressure noted above, should be sufficient to produce a substantial improvement in the properties of the lubricating oil being treated. Generally speaking, this time will range from 15 to 150 minutes. A period of time ranging from 110 to 130 minutes is often preferred and is used in the examples.

It is preferred that the substantially anhydrous hydrofluoric acid be the major or dominating component of the reaction mixture, i. e., that it be present in greater amount than any other component. It is desirable to use such proportions that the hydrofluoric acid is present in the greatest amount with the naphthene next in amount and the oil least in amount. Preferred proportions are those wherein the amount of hydrofluoric acid ranges from 1.6 to 2.0 times the weight of the oil and the amount of naphthene ranges from 1.3 to 1.7 times the weight of the oil, the amount of hydrofluoric acid substantially exceeding the amount of naphthene. These proportions are, however, not critical, but it is distinctly advantageous to use sufficient hydrofluoric acid to form a separate acid phase.

Generally the materials present in the reaction

zone will consist of the oil, the anhydrous liquid hydrofluoric acid and the naphthene. Of course, other materials formed as by-products and present in the recycle streams described more fully below may be present in the reaction zone. I refer in particular to low molecular weight cycloalkyl hydrocarbons which are recovered from the reaction mixture and advantageously recycled together with unreacted naphthene.

However, I do not wish to exclude the use of a diluent in the reaction zone. Such a diluent will generally be a condensable paraffin, usually a liquid paraffin such as liquid propane, liquid normal butane or normal pentane or normal hexane. As disclosed more fully below, in a modification of the present invention I may use an aliphatic paraffin, particularly an aliphatic isoparaffin and especially an aliphatic C<sub>4</sub> to C<sub>6</sub> isoparaffin as a component of the reaction mixture to produce certain advantageous results noted below. Such an aliphatic paraffin may, of course, additionally serve to dilute and render less viscous the reaction mixture.

Other than by-products such as cycloalkyls which may be present in certain recycle streams as noted above, however, the reaction mixture will consist of the lubricating oil to be treated, the liquid hydrofluoric acid, and the naphthene, an aliphatic paraffin being optionally present, all other materials being excluded from the reaction system.

The amount of hydrofluoric acid is almost invariably such that a separate acid phase is present in the reaction zone. Any suitable equipment for carrying out the reaction may be employed. Generally, however, the equipment will be so designed as to provide intimate contacting between the acid and the hydrocarbon phases throughout the reaction period. The contacting equipment may be similar to or identical with the contactors which are commonly used for conducting the alkylation of aliphatic isoparaffins with aliphatic olefins. An example is the so-called "Stratco" contactor. Any other means of maintaining a fine emulsion of the acid and hydrocarbon phases may be employed. The equipment used should be provided with means for maintaining the elevated temperature desired for the reaction. This means may take the form of indirect heating arrangements of known type.

Following agitation of the reaction mixture for the selected contact time at the elevated temperature and pressure employed, the reaction mixture may be withdrawn from the reaction zone and allowed to cool and settle, usually by gravity, into two separate layers, namely, a lower acid layer and an upper hydrocarbon layer. These layers are separated in any suitable manner. The treated lubricating oil may then be recovered from the hydrocarbon layer. For example, the hydrocarbon layer may be washed with dilute caustic solution and then topped under vacuum to the initial boiling point of the untreated lubricating oil to remove low-boiling constituents.

Generally, however, it will be preferred to subject the hydrocarbon layer to vacuum fractionation to recover a light fraction containing unreacted naphthene and low molecular weight cycloalkyl hydrocarbons, produced as by-products in the reaction, from a bottoms fraction of the treated lubricating oil. This bottoms fraction may then be washed with dilute caustic solution to give the finished oil. The acid layer comprises hydrofluoric acid containing in solution acid-soluble oils derived from the original oil and

formed as by-products during the reaction. I prefer to fractionally distill this acid layer to separate it into a light overhead fraction of the hydrofluoric acid and a bottoms fraction of the acid-soluble oils. This bottoms fraction is discarded from the system. The hydrofluoric acid overhead is preferably recycled as a source of hydrofluoric acid for the reaction.

The process may be carried out either in a batchwise manner or continuously, the latter 10 being preferred for commercial operation.

I have found that when particular lubricating oils, such as those derived from mixed-base crudes, are treated with liquid anhydrous hydrofluoric acid and a naphthene, particularly cyclohexane, product oils with high stability and high viscosity indices result, but the oils are darker than the original oils and have an undesirably high cloud point. I have found, however, that this undesirable effect may be overcome by using 20 an aliphatic paraffin in conjunction with the naphthene.

In accordance with the latter aspect of my invention, lubricating oils of high stability, high viscosity index, improved color and low cloud point may be obtained by treating lubricating oils, especially mixed-base lubricating oils, with a mixture consisting of liquid anhydrous hydrofluoric acid, an aliphatic paraffin, particularly an aliphatic isoparaffin, and especially an aliphatic isoparaffin having from four to six carbon atoms per molecule, and a naphthene, particularly cyclohexane.

Any aliphatic C<sub>4</sub> to C<sub>6</sub> paraffin may be employed in this modification of my invention but I prefer an isoparaffin, namely, either isobutane, isopentane or isohexane. Isopentane is preferred. The conditions of treatment are the same as those given above in detail for the treatment with hydrofluoric acid and a naphthene alone.

When an aliphatic paraffin, such as a C<sub>4</sub> to C<sub>6</sub> isoparaffin, is used, the total amount of aliphatic paraffin plus naphthene may range from 1.3 to 1.7 times the weight of the oil. Amounts beyond these limits may, however, be effectively used if desired. The proportion of the aliphatic paraffin in the combined aliphatic paraffin plus naphthene may range from 0 to 60 per cent by weight, but is preferably from 40 to 60 per cent by weight of the total amount of naphthene plus isoparaffin. Ordinarily, approximately equal volumes of the naphthene and the isoparaffin will be employed. The proportion of hydrofluoric acid employed may be the same as that given above, namely, from 1.6 to 2.0 times the weight of the oil, but other proportions may be effectively used, provided that sufficient acid is present to form a separate liquid phase.

Preferably this embodiment of my invention is conducted by using isopentane in conjunction with cyclohexane for the modification of the lubricating oil. Ordinarily, approximately equal volumes of isopentane and cyclohexane are employed.

In another aspect of my invention, I use methylcyclopentane as the naphthene. I have found that when certain lubricating oils, particularly those derived from mixed-base crudes, are treated with liquid anhydrous hydrofluoric acid and a naphthene other than methylcyclopentane such as cyclohexane, cyclopentane, decalin, methylcyclohexane, etc., or with hydrofluoric acid and a mixture of an aliphatic paraffin and a naphthene such as a mixture of isopentane and cyclohexane,

product oils of high viscosity index and improved stability are obtained. However, the viscosity of the product oil is generally less than that of the original oil. Also from 6 to 9 per cent of the treated oil is converted to acid-soluble material, which represents a loss of material and is a relatively undesirable by-product of the process.

I have found, however, that when methylcyclopentane is the naphthene employed for the treatment, these objections are overcome. For example, upon treatment of a mixed-base lubricating oil with hydrofluoric acid and methylcyclopentane in accordance with my invention, the lubricating oil produced has high stability, high viscosity index and increased viscosity. Yet only a small portion of the oil is converted to acid-soluble oil. The conditions and proportions given above apply equally to this modification of my invention.

Although the chemical changes that take place when a mixed-base lubricating oil is treated with anhydrous liquid hydrofluoric acid and methylcyclopentane are not thoroughly understood, I believe that the predominant reaction is alkylation in which methylcyclopentane is alkylated by products of disproportionation of relatively unstable material in the oil which otherwise would be converted to acid-soluble oil. The fact that this effect is not as pronounced with other naphthenes, such as cyclopentane, methylcyclohexane, cyclohexane and decalin, indicates that methylcyclopentane is alkylated more easily by certain constituents of the oil. In treating oil with liquid anhydrous hydrofluoric acid and methylcyclopentane, the same conditions and proportions of reactants which are given in detail above are employed.

In particular instances, it may be advantageous to treat the lubricating oils with a mixture of naphthenes, such as cyclohexane and methylcyclopentane, whereby oils of high viscosity index and stability are obtained with a minimum of oil being converted to acid-soluble oil. Mixtures of two or more naphthenes and an aliphatic paraffin may also be used.

As mentioned above, the process of my invention is applicable not only to natural lubricants but also to synthetic lubricating oils produced by polymerizing olefins. One disadvantage of some such synthetic lubricating oils is that their viscosity index is comparatively low. Treatment of such olefin polymers with liquid anhydrous hydrofluoric acid and a naphthene, such as cyclopentane, methylcyclopentane, cyclohexane and methylcyclohexane, yields a lubricant having increased viscosity index and degree of saturation.

One example of a synthetic oil is the type produced by polymerizing low-boiling aliphatic olefins of at least three carbon atoms per molecule 60 with a zirconium tetrahalide catalyst under controlled conditions as taught in U. S. Patent to Reid, No. 2,389,240.

The conditions for treatment of olefin polymer in accordance with this invention are, in general, 65 the same as those previously described for treatment of natural lubricating oils and the considerations advanced above apply. The same ranges of relative proportions are employed. The optimum conditions in any given instance depend on 70 the nature of the specific polymer treated and the specific naphthene used, and can readily be determined by trial. In many cases the temperature of treatment will cover a lower range, say from 40 to 200° C. instead of 40 to 300° C. as given 75 for the natural oils.

Following are specific examples of the treatment of lubricating oils with hydrofluoric acid in the presence of a naphthalene or a mixture of naphthalene and aliphatic paraffin. The procedure employed in Examples 1 to 6 was as follows.

A 4.5-liter steel bomb was charged with liquid anhydrous hydrofluoric acid, a mixed-base lubricating oil, a cycloparaffin, and, when desired, an aliphatic paraffin. The charged bomb was clamped to a rocker and was fitted with a suitable pressure gauge. The bomb was heated and agitated for the desired time and was removed from the rocker and placed in a vertical position. The contents of the bomb were allowed to cool and settle. The acid and hydrocarbon layers were separated, and the hydrocarbon layer was washed with dilute caustic solution. The acid layer was heated to remove hydrofluoric acid, and the residue was weighed. The hydrocarbon layer was then topped to 450° F. at approximately 2 to 3 mm. pressure (the initial boiling point of the untreated oil) to remove low-boiling constituents.

The following data were obtained:

#### EXAMPLES 1 TO 6

|                                 | Untreated Oil | Example            |             |             |         |              |                     |
|---------------------------------|---------------|--------------------|-------------|-------------|---------|--------------|---------------------|
|                                 |               | 1                  | 2           | 3           | 4       | 5            | 6                   |
| Oil, grams                      | 527.          | 524.               | 530.        | 524.        | 527.    | 524.         |                     |
| HF, grams                       | 1031.         | 1022.              | 990.        | 922.        | 917.    | 963.         |                     |
| Aliphatic paraffin              |               |                    |             |             |         |              |                     |
| Aliphatic paraffin, gms.        |               |                    | 319.        |             |         |              |                     |
| Cycloparaffin                   |               | Methylcyclohexane. | Cyclohexane | Cyclohexane | Decalin | Cyclopentane | Methylcyclopentane. |
| Cycloparaffin, grams            | 754.          | 766.               | 378.        | 879.        | 730.    | 752.         |                     |
| Contact time, minutes           | 120.          | 120.               | 120.        | 120.        | 120.    | 120.         |                     |
| Maximum temperature, °C         | 150.          | 148.               | 151.        | 163.        | 156.    | 154.         |                     |
| Maximum pressure, p. s. i.      | 650.          | 670.               | 730.        | 660.        | 840.    | 730.         |                     |
| Weight percent acid-solubles    | 6.            | 8.                 | 7.          | 9.          | 9.      | 3.           |                     |
| <i>Test Data</i>                |               |                    |             |             |         |              |                     |
| Viscosity, 100° F., SUS         | 287.3         | 265.1              | 245.2       | 235.4       | 269.8   | 236.6        | 306.8.              |
| Viscosity, 210° F., SUS         | 50.77         | 50.37              | 49.77       | 48.98       | 50.30   | 48.88        | 52.63.              |
| Viscosity Index (Dean & Davis). | 89            | 98                 | 104         | 102         | 94      | 100          | 96.                 |
| Cloud Point, °F                 | +32           | +36                | +72         | +36         | +72     | +30          | +30.                |
| Pour Point, °F                  | +30           | +30                | +35         | +30         | +35     | +30          | +30.                |
| API Gravity                     | 28.7          | 30.3               | 30.1        | 30.7        | 29.2    | 30.5         | 30.4.               |
| ASTM Color                      | 2½            | 2+                 | 3½          | 2½          | 3       | 3½           | 2½.                 |

Inspection of the data obtained shows that when a mixed-base lubricating oil is treated with hydrofluoric acid and a naphthalene, an oil with a substantially increased viscosity index is obtained. From Example 4, it appears that decalin gives the least improvement in viscosity index. Comparison of the data given for Example 6 with the other examples shows that when methylcyclopentane is used, both the viscosity and the viscosity index are substantially increased and yet a minimum amount of acid-solubles is produced. The data for the other examples indicate that this effect is not shown by the other naphthalenes studied or by a mixture of an aliphatic paraffin and a cycloparaffin (Example 3).

Comparison of the data obtained in Example 3 with those obtained in Example 2 shows that the product oil from Example 3 has a considerably lower cloud point, a lower pour point and a lower ASTM color than the oil from Example 2. The data for Example 1 show that treatment of a mixed-base lubricating oil with hydrofluoric acid and methylcyclohexane does not raise the cloud point materially. The viscosity index for the product oil from Example 3 is greater than that for the oil from Example 1.

Samples of the untreated oil and the product oil from Example 2 were vacuum fractionated and the viscosity index and refractive index of each fraction were determined. The data set forth in Table A were obtained.

These data show that treatment of the oil with HF and cyclohexane produces a considerable chemical change in the oil.

Aluminum block stability data obtained for the untreated oil and the product oils from Examples 2 (blend of fractions 1 through 6) and 6 are tabulated as follows:

Table B

|                                                           | Untreated Oil | Example     |                    |
|-----------------------------------------------------------|---------------|-------------|--------------------|
|                                                           |               | 1           | 2                  |
| Naphthalene used                                          |               | Cyclohexane | Methylcyclopentane |
| Evaporation loss, wt. percent                             | 4.3           | 1.7         | 1.3                |
| Neutralization number:                                    |               |             |                    |
| before heating                                            | 0.00          | 0.01        | 0.02               |
| after heating                                             | 0.33          | 0.13        | 0.28               |
| Ramsbottom carbon residue, wt. percent:                   |               |             |                    |
| before heating                                            | 0.02          | 0.04        | 0.05               |
| after heating                                             | 0.21          | 0.04        | 0.15               |
| Naphthalene insolubles, wt. percent: after heating        | 0.08          | 0.00        | 0.07               |
| Percent Viscosity increase corrected for evaporation loss | 5.2           | 2.5         | 4.2                |

These data show that the HF-cyclohexane and HF-methylcyclopentane treated oils have greater stability than the untreated oil.

**9**  
**EXAMPLE 7**

This example shows the results of treatment of an olefin polymer in accordance with the present invention. This example consists of two parts, namely, Part A which includes the preparation of the olefin polymer, and Part B which includes the treatment of the olefin polymer with hydrofluoric acid and methylcyclohexane.

*A.—Preparation of Olefin Polymer*

An 18-liter steel reactor provided with a mechanical stirrer was charged with 450 grams of zirconium tetrachloride catalyst and 1 gallon of normal pentane. Thirteen and four-tenths pounds of propylene was gradually added to the reactor over an 8-hour period. The mixture was stirred for an additional 4 hours. The average temperature was 130° F. The pressure at the end of the run was 30 pounds per square inch.

The reactants were allowed to stand, without stirring, until the catalyst separated from the hydrocarbon. The hydrocarbon was then decanted from the catalyst. The hydrocarbon was filtered through a filter aid and was depentanized. The resulting polymer was topped in a flash chamber. The material which distilled from 455° F. at 20 mm. to 527° F. at 0.1 mm. was collected.

*B.—Treatment of olefin polymer in accordance with the invention*

Four hundred ninety-eight grams of the polymer as produced in A, 1151 grams of methylcyclohexane, and 1026 grams of commercial anhydrous hydrofluoric acid were charged to a 4.5-liter steel bomb. The charged bomb was clamped to a platform rocker and was fitted with a suitable pressure gauge. The bomb was continuously heated and agitated for 120 minutes. The maximum temperature was 151° C.; maximum pressure, 635 pounds per square inch. The bomb was removed from the rocker and placed in a vertical position. The bomb contents were allowed to cool and settle and the acid and hydrocarbon layers were separated. The hydrocarbon layer was washed with dilute caustic solution and was separated and dried. After filtering through a filter aid, the product hydrocarbon was topped at 450° F. and 5 mm. The following test data were obtained:

|                                | Untreated Polymer | Hydrofluoric Acid-Methylcyclohexane-Treated Polymer |
|--------------------------------|-------------------|-----------------------------------------------------|
| Viscosity, 100° F., SUS        | 449.6             | 279.9                                               |
| Viscosity, 210° F., SUS        | 54.11             | 48.37                                               |
| Viscosity Index (Dean & Davis) | 48                | 62                                                  |
| Pour Point, ° F.               |                   | -30                                                 |
| API Gravity                    | 37.2              | 38.2                                                |
| ASTM Color                     |                   | 1                                                   |
| Refractive Index (20° C.)      | 1.4681            | 1.4620                                              |

In the drawing, the reactor 1 is charged with lubricating oil to be treated by means of line 2, with anhydrous hydrofluoric acid via line 3, and with naphthene hydrocarbon via line 4. If an aliphatic paraffin is to be employed in the treatment, it is charged via line 5. The reactants are agitated in reactor 1 for a selected contact time at elevated temperature and pressure. From reactor 1 the reaction mixture composed of hydrofluoric acid, and residue, lubricating oil, by-product low molecular weight cycloalkyl compounds, and naphthene hydrocarbon, and aliphatic paraffin if that was used, is passed to sep-

**10**

arator 6 which may be of a type such as is known for the separation of the effluent from the hydrofluoric acid ankylation of isoparaffins with aliphatic olefins. In separator 6 the acid and hydrocarbon layers are separated, usually by means of gravity. The acid layer is passed via line 7 to fractionator 8 wherein it is separated into an overhead fraction of hydrofluoric acid which is recycled via line 9 and a bottoms fraction of acid residue which is withdrawn via line 10. The acid residue consists of the acid-soluble material dissolved by the acid in the reactor 1.

The hydrocarbon layer from separator 6 is passed via line 11 to vacuum fractionation column 12. Naphthene and low molecular weight cycloalkyls may be separated and recycled via line 13. If an aliphatic paraffin was charged to reactor 1, a stream of unreacted aliphatic paraffin may be withdrawn from vacuum fractionator 12 and recycled via line 14. Lubricating oil from vacuum fractionator 12 is withdrawn via line 15 as a product of the process. If desired, the product oil may be washed with caustic solution to remove hydrofluoric acid.

It will be understood that vacuum column 12 and the takeoff lines 13 and 14 are shown merely diagrammatically. If an aliphatic paraffin was charged, it may be desirable to recover a single overhead fraction containing the unreacted aliphatic paraffin, naphthene and the low molecular weight cycloalkyl compounds and to recycle these without separation. However, better control over the reaction may be obtainable by separately recovering and recycling the two fractions shown in lines 13 and 14 since such separate recycle enables more accurate metering of reactants to reactor 1.

From the foregoing description, it will be seen that the present invention provides a simple and economical process for improving lubricating oils. The process is particularly valuable for the improvement of mixed-base lubricating oils which in the past have been considered to have certain disadvantages relative to paraffin-base lubricating oils, although it was recognized that mixed-base oils had certain advantages not possessed by the paraffin-base oils.

Specifically, the present invention enables a substantial increase in viscosity index and stability of the oil to be brought about. The invention also enables olefin polymer types of synthetic lubricating oil to be improved materially.

I claim:

1. The process of improving lubricating oil which comprises contacting said lubricating oil with substantially anhydrous liquid hydrofluoric acid in proportion sufficient to form a separate acid phase and with an added naphthene selected from a group consisting of cyclopentane, methylcyclopentane, cyclohexane, and methylcyclohexane in an amount ranging from 1.3 to 1.7 times the weight of said oil at elevated temperature of from 40 to 300° C. at a pressure sufficient to maintain the hydrofluoric acid and hydrocarbons in liquid phase for a period of time sufficient to produce a substantial increase in the viscosity index and stability of said lubricating oil, and recovering the treated lubricating oil from the resulting reaction mixture.
2. The process of improving lubricating oil which comprises contacting said lubricating oil with substantially anhydrous liquid hydrofluoric acid in proportion sufficient to form a separate acid phase and with added methylcyclohexane in an amount ranging from 1.3 to 1.7 times the

## 11

weight of the oil at elevated temperature of from 40 to 300° C. and at a pressure sufficient to maintain the hydrofluoric acid and hydrocarbons in liquid phase for a period of time sufficient to produce a substantial increase in the viscosity index and stability of said lubricating oil, and recovering the treated lubricating oil from the resulting reaction mixture.

3. The process of improving lubricating oil which comprises contacting said lubricating oil with substantially anhydrous liquid hydrofluoric acid in proportion sufficient to form a separate acid phase and with added cyclohexane in an amount ranging from 1.3 to 1.7 times the weight of the oil at elevated temperature of from 40 to 300° C. and at a pressure sufficient to maintain the hydrofluoric acid and hydrocarbons in liquid phase for a period of time sufficient to produce a substantial increase in the viscosity index and stability of said lubricating oil, and recovering the treated lubricating oil from the resulting reaction mixture.

4. The process of improving lubricating oil which comprises contacting said lubricating oil with substantially anhydrous liquid hydrofluoric acid in proportion sufficient to form a separate acid phase and with added methylcyclopentane in an amount ranging from 1.3 to 1.7 times the weight of the oil at elevated temperature of from 40 to 300° C. and at a pressure sufficient to maintain the hydrofluoric acid and hydrocarbons in liquid phase for a period of time sufficient to produce a substantial increase in the viscosity index and stability of said lubricating oil, and recovering the treated lubricating oil from the resulting reaction mixture.

5. The process of improving lubricating oil which comprises contacting said lubricating oil with substantially anhydrous liquid hydrofluoric acid in proportion sufficient to form a separate acid phase and with added naphthene selected from a group consisting of cyclopentane, methylcyclopentane, cyclohexane, and methylcyclohexane in an amount greater than said lubricating oil while maintaining a temperature of from 40 to 300° C. and a pressure sufficient to maintain the hydrofluoric acid and the hydrocarbons in liquid phase for a period of time ranging from 15 to 150 minutes and sufficient to produce a substantial increase in the viscosity index and stability of said lubricating oil, and recovering the treated lubricating oil from the resulting reaction mixture.

6. The process of improving lubricating oil which comprises contacting said lubricating oil with substantially anhydrous liquid hydrofluoric acid in proportion sufficient to form a separate acid phase and with added naphthene selected from a group consisting of cyclopentane, methylcyclopentane, cyclohexane, and methylcyclohexane in an amount greater than said lubricating oil while maintaining a temperature of from 140 to 170° C. and a pressure sufficient to maintain the hydrofluoric acid and the hydrocarbons in liquid phase for a period of time ranging from 110 to 130 minutes and sufficient to produce a substantial increase in the viscosity index and stability of said lubricating oil, and recovering the treated lubricating oil from the resulting reaction mixture.

7. The process of improving lubricating oil which comprises subjecting a mixture consisting of said lubricating oil, substantially anhydrous liquid hydrofluoric acid and an added naphthene selected from a group consisting of cyclopentane,

## 12

methylcyclopentane, cyclohexane, and methylcyclohexane, the proportions in said mixture being such that the hydrofluoric acid is greatest in amount, the naphthene is next in amount and the oil is least in amount, to an elevated temperature of from 40 to 300° C. and a pressure sufficient to maintain the hydrofluoric acid and the hydrocarbons in liquid phase for a period of time ranging from 15 to 150 minutes and sufficient to produce a substantial increase in the viscosity index and stability of said lubricating oil, and recovering the treated lubricating oil from the resulting reaction mixture.

8. The process of improving lubricating oil which comprises subjecting a mixture consisting of said lubricating oil, substantially anhydrous liquid hydrofluoric acid and an added naphthene selected from a group consisting of cyclopentane, methylcyclopentane, cyclohexane, and methylcyclohexane, the proportions in said mixture being such that the amount of hydrofluoric acid ranges from 1.6 to 2.0 times the weight of said oil and the amount of naphthene ranges from 1.3 to 1.7 times the weight of said oil, to a temperature of from 140 to 170° C. and a pressure sufficient to maintain the hydrofluoric acid and the hydrocarbons in liquid phase for a period of time ranging from 110 to 130 minutes and sufficient to produce a substantial increase in the viscosity index and stability of said lubricating oil, and recovering the treated lubricating oil from the resulting reaction mixture.

9. The process of improving mixed-base lubricating oil which comprises contacting said mixed-base lubricating oil with substantially anhydrous liquid hydrofluoric acid in proportion sufficient to form a separate acid phase and with added methylcyclopentane in an amount greater than said lubricating oil while maintaining a temperature of from 100 to 200° C. and a pressure sufficient to maintain the hydrofluoric acid and the hydrocarbons in liquid phase for a period of time ranging from 15 to 150 minutes and sufficient to produce a substantial increase in the viscosity index, viscosity and stability of said lubricating oil, and recovering the treated lubricating oil from the resulting reaction mixture.

10. The process of improving lubricating oil which comprises contacting said lubricating oil with substantially anhydrous liquid hydrofluoric acid in proportion sufficient to form a separate acid phase and with an added C<sub>4</sub> to C<sub>6</sub> aliphatic paraffin and an added naphthene selected from a group consisting of cyclopentane, methylcyclopentane, cyclohexane, and methylcyclohexane in an amount such that the total amount of aliphatic paraffin plus naphthene ranges from 1.3 to 1.7 times the weight of said lubricating oil and the amount of said aliphatic paraffin ranges up to 60 per cent by weight of the amount of added aliphatic paraffin plus added naphthene at elevated temperature of from 40 to 300° C. and at a pressure sufficient to maintain the hydrofluoric acid and hydrocarbons in liquid phase for a period of time sufficient to produce a substantial increase in the viscosity index and stability of said lubricating oil, and recovering the treated lubricating oil from the resulting reaction mixture.

11. The process of improving mixed-base lubricating oil which comprises contacting said mixed-base lubricating oil with substantially anhydrous liquid hydrofluoric acid in proportion sufficient to form a separate acid phase and with added isopentane and added cyclohexane in an

**13**

amount such that said isopentane plus cyclohexane ranges from 1.3 to 1.7 times the weight of said lubricating oil and the amount of said added isopentane ranges from 40 to 60 per cent by weight of the amount of added isopentane plus added naphthene at elevated temperature of from 40 to 300° C. and pressure sufficient to maintain the hydrofluoric acid and hydrocarbons in liquid phase for a period of time sufficient to produce a substantial increase in the viscosity index and stability of said lubricating oil, and recovering the treated lubricating oil from the resulting reaction mixture. 10

12. The process of improving synthetic lubricating oil produced by polymerizing olefins which comprises contacting said synthetic lubricating oil with substantially anhydrous hydrofluoric acid in proportion sufficient to form a separate acid phase and an added naphthene selected from a group consisting of cyclopentane, methylcyclopentane, cyclohexane, and methylcyclohexane in an amount ranging from 1.3 to 1.7 times 20

**14**

the weight of said oil while maintaining a temperature of from 40 to 200° C. and a pressure sufficient to maintain the hydrofluoric acid and the hydrocarbons in liquid phase for a period of time ranging from 15 to 150 minutes and sufficient to produce a substantial increase in the viscosity index and degree of saturation of said lubricating oil, and recovering the treated lubricating oil from the resulting reaction mixture.

PAUL H. CARNELL.

**REFERENCES CITED**

The following references are of record in the file of this patent:

**UNITED STATES PATENTS**

| Number    | Name     | Date          |
|-----------|----------|---------------|
| 2,320,629 | Matuszak | June 1, 1943  |
| 2,366,743 | Matuszak | Jan. 9, 1945  |
| 2,375,675 | Matuszak | May 8, 1945   |
| 2,378,762 | Frey     | June 19, 1945 |